

R. F. BACON.  
METALLURGY OF COPPER.  
APPLICATION FILED MAR. 20, 1915.

1,151,236.

Patented Aug. 24, 1915.



Witnesses:

M. Anna

J. Nathan

Inventor:

Raymond F. Bacon

By  
Pennie Davis & Marvin  
Attys.

# UNITED STATES PATENT OFFICE.

RAYMOND F. BACON, OF PITTSBURGH, PENNSYLVANIA, ASSIGNOR TO METALS  
RESEARCH COMPANY, OF NEW YORK, N. Y., A CORPORATION OF MAINE.

## METALLURGY OF COPPER.

1,151,236.

Specification of Letters Patent. Patented Aug. 24, 1915.

Application filed March 20, 1915. Serial No. 15,857.

To all whom it may concern:

Be it known that I, RAYMOND F. BACON, residing at and whose post-office address is Pittsburgh, Allegheny county, State of Pennsylvania, have invented certain new and useful Improvements in Metallurgy of Copper; and I do hereby declare the following to be a full, clear, and exact description of the invention, such as will enable others skilled in the art to which it appertains to make and use the same.

The present invention relates to certain new and useful improvements in the hydro-metallurgy of copper and particularly to the recovery of copper from solutions of copper salts, such as are obtained by the lixiviation of copper ores and furnace residues by means of sulfuric acid or hydrochloric acid, or such as are present in mine waters and the like.

The practice of the invention, in its preferred form, involves a process wherein, first, hydrogen sulfid is produced by reaction, at a relatively low temperature, between sulfur and a hydrocarbon; secondly, wherein a portion of the hydrogen sulfid reacts with sulfur dioxid to produce a quantity of sulfur equal in amount to that which is utilized in the first step of the operation; thirdly, wherein the remainder of the hydrogen sulfid produced in the first step of the operation is employed for the precipitation of copper sulfid from the copper salt solution (say a solution of copper sulfate or copper chlorid), and with the simultaneous restoration of sulfuric acid to the solution; and fourthly, wherein the copper sulfid is roasted, the resulting sulfur dioxid fumes being thereupon utilized in the second step of the process. The solution from which the copper has been precipitated in the form of copper chlorid and which, as the result of the reaction has had its sulfuric acid or hydrochloric acid regenerated therein, may be employed for the lixiviation of a further quantity of ore or the like.

In order to produce a quantity of hydrogen sulfid adapted to the convenient and efficient employment of the process, elemental sulfur, (as, for instance, precipitated sulfur from a former operation) is treated with a hydrocarbon, as, for instance, what is known as hydrocarbon residue, and at a temperature which may conveniently be that of the

boiling point of the hydrocarbon employed, 55 which, in the case of hydrocarbon residue, would vary from say 300° C. to 360° C. The temperature employed should not materially exceed the boiling point of the hydrocarbon, for the reason that hydrogen sulfid 60 begins to dissociate at a temperature of about 400° C. and such dissociation becomes increasingly important at higher temperatures, so that it is preferable to restrict the temperature accordingly, not permitting 65 it to rise above say 500° C. So also, it is found preferable to employ a quantity of hydrocarbon not materially exceeding and closely approaching the quantity required to satisfy the contemplated reaction, for the 70 reason that when the amount of hydrocarbon is thus restricted, the coke (which, with the hydrogen sulfid is the product of the reaction) is found to be harder and denser, and therefore better adapted for most of the 75 uses for which coke is intended,—particularly as a constituent of the charge of a blast furnace or the like, i. e., as metallurgical coke. The reaction involving this simultaneous production of hydrogen sulfid and 80 coke may be expressed by the following general equation:



A part of the hydrogen sulfid thus produced, may then be caused to react with sulfur dioxid, which latter is derived from the subsequent roasting step of the cyclic process. The SO<sub>2</sub> gases are either employed in their gaseous condition, as they come from the roasting furnace, or they may be absorbed in water and treated by passing the hydrogen sulfid into the water in which the SO<sub>2</sub> has been absorbed. The resulting reaction may be expressed by the following 95 general formula:



Another portion of the hydrogen sulfid produced in the first step of the operation 100 is then employed to precipitate the copper, in the form of copper sulfid, from the copper salt solution, which latter, as hereinbefore stated, may be obtained from any suitable available source, as, for instance, by 105 lixiviating copper ores with sulfuric acid or hydrochloric acid, or which may be available as mine waters holding a copper salt in

solution. The resulting reaction may be expressed by the following formula:



5 The resulting spent solution containing the regenerated sulfuric acid or hydrochloric acid, as the case may be, may be employed for the lixiviation of a further body of ore. The copper sulfid resulting from 10 the third step of the operation is then roasted, with the production of copper oxid, and of sulfur dioxid in the products of combustion, in accordance with the following formula:



It will now be evident that the  $\text{SO}_2$  gases thus produced are available for re-use in the second step of the operation. Accordingly, 20 the procedure described permits the constant reutilization, in the cycle, of the sulfur dioxid fumes given off in the roasting operation, and, as hereinbefore pointed out, the elemental sulfur produced in the second step 25 of the operation is utilizable for the production of further quantities of hydrogen sulfid; so that the procedure involves a self-sustaining operation in its several steps, in the sense that the hydrogen sulfid, the sulfur, and the sulfur dioxid produced in the 30 several stages are utilized in subsequent stages thereof. The ultimate products of the operation consist of copper oxid, and a high grade of coke, and, if desired, the coke 35 may be employed for the reduction of the copper oxid to metallic copper. So also,

as hereinbefore pointed out, the copper solution treated is regenerated and therefore made available for the lixiviation of a further quantity of ore.

40

In the accompanying drawing are represented, for convenience of reference, in appropriate grouping, the reactions characterizing the practice of the invention.

Having thus described my invention, what 45 I claim is:

The method of carrying on a cyclic operation for the recovery of copper from solutions containing it, which consists first, in producing hydrogen sulfid; secondly, producing elemental sulfur by reaction between sulfur dioxid and a portion of said hydrogen sulfid; thirdly, employing the remaining portion of the hydrogen sulfid for precipitating the copper, as copper sulfid, from the 50 copper salt solution to be treated while simultaneously regenerating the solution; fourthly, roasting the copper sulfid, with the simultaneous production of sulfur dioxid; the elemental sulfur and the sulfur dioxid 55 produced in the second and fourth stages, respectively, being subsequently utilized in maintaining a cyclic operation, *i. e.*, by using said sulfur in a recurrent first stage, and said sulfur dioxid in a recurrent second 60 stage thereof; substantially as described.

In testimony whereof I affix my signature, in presence of two witnesses.

RAYMOND F. BACON.

Witnesses:

KATHARINE SCHULZ,  
M. A. BILL.